

# UNITED STATES PATENT OFFICE

FRIEDRICH EMIL DIETLER, OF KELSTERBACH-ON-THE-MAIN, GERMANY, ASSIGNOR TO VEREINIGTE KUNSTSEIDEFAERIEN A. G., OF KELSTERBACH-ON-THE-MAIN, GERMANY, A CORPORATION OF GERMANY.

## PROCESS OF MANUFACTURING ARTIFICIAL LUSTROUS THREADS, &c.

1,121,903.

Specification of Letters Patent. Patented Dec. 22, 1914.

No Drawing.

Application filed June 18, 1912. Serial No. 704,269.

*To all whom it may concern:*

Be it known that I, FRIEDRICH EMIL DIETLER, a subject of the German Emperor, residing at Kelsterbach-on-the-Main, in the 5 German Empire, have invented certain new and useful Improvements in Processes of Manufacturing Artificial Lustrous Threads, &c., of which the following is a specification.

My invention is concerned with methods 10 of producing highly lustrous threads, filaments and like articles from viscose, and relates particularly to the composition of the precipitation bath employed in one of the steps of the method.

15 The use of an acidulated bath for the production of water soluble xanthogenate threads from viscose and the subsequent conversion of the xanthogenate into water insoluble cellulose hydrate has been heretofore suggested. No indication, however, was given as to the nature of the bath to be employed, nor was there any hint of the quantity of acid to be introduced in order to produce commercially satisfactory, lustrous, 20 threads. Extensive experiments have shown that it is not always possible to produce commercially satisfactory, lustrous threads, by treating such threads in a bath consisting of a saturated salt solution to which acid has 25 been added. If, for example, sulfuric acid is employed and sodium bisulfate is dissolved therein, so that the content of free sulfuric acid amounts to about 20%, experiments have demonstrated that a bath of this kind will effect an immediate conversion of the viscose into water insoluble cellulose hydrate, but the thread treated will not be lustrous. If the addition of the sulfuric acid to the saturated sodium sulfate solution is less 30 in quantity, for example 6 to 7%, there is no conversion of the viscose into water insoluble cellulose hydrate, there is merely a removal of salts from the viscose. There are, however, sulfurous exudations in the form of a bluish glint in the outer strata of the product. If the sulfur is dissolved out, dull places remain which decrease the luster of the final product. By acidulating the saturated salt solution with but a small quantity of sulfuric acid, for example 0.5%, the precipita- 35

tion (salt removal) proceeds too slowly. The several disadvantages above referred to are obviated, as I have ascertained, if the quantity of sulfuric acid added to the salt solution is between 1 and 5%.

55 A bath according to my invention may be prepared as follows:—Dissolve 10 parts of neutral sodium sulfate in 100 parts of water, and add to this salt solution 1 to 5 parts of sulfuric acid, 1.84 specific gravity. The bath 60 thus produced not only effects a rapid precipitation of the xanthogenate, but, moreover, there are no sulfurous exudations on the surface of the product. To convert the product into water insoluble cellulose hydrate it is subjected to the usual treatment of heating, treatment in a bath of common salt, etc. The product finally obtained is 65 highly lustrous, strong and elastic.

70 I claim:—

1. The herein described process of manufacturing artificial, lustrous threads, bands and filaments, which consists in forming viscose solution into thread like bodies, and thereafter subjecting the same to the action 75 of a precipitation bath consisting of a salt solution containing not exceeding five per centum of acid.

2. The herein described process of manufacturing artificial, lustrous threads, bands 80 and filaments, which consists in forming viscose solution into thread like bodies, and thereafter subjecting the same to the action of a precipitation bath consisting of a saturated salt solution containing not exceeding 85 five per centum of sulfuric acid.

3. The herein described process of manufacturing artificial, lustrous threads, bands and filaments, which consists in forming viscose solution into thread like bodies, and 90 thereafter subjecting the same to the action of a precipitation bath consisting of a solution of ten parts of neutral sodium sulfate in one hundred parts of water, and not exceeding five parts of sulfuric acid of 1.84 95 specific gravity.

4. The herein described process of manufacturing artificial, lustrous threads, bands and filaments, which consists in forming viscose solution into thread like bodies, there- 100

after subjecting the same to the action of a precipitation bath consisting of a solution of ten parts of neutral sodium sulfate in one hundred parts of water and not exceeding 5 five parts of sulfuric acid of 1.84 specific gravity, and finally converting the product into water insoluble cellulose hydrate.

In testimony whereof I have affixed my signature in presence of two witnesses.

FRIEDRICH EMIL DIETLER.

Witnesses:

JEAN GRUND,  
CARL GRUND.